# EUROPEAN PATENT SPECIFICATION

(11) **EP 1 084 830 B1**
(45) Date of publication and mention of the grant of the patent: **02.07.2003**
(21) Application number: 99203064.3
(22) Date of filing: 15.09.1999
(51) Int. Cl.: B41C 1/10

(54) **Method for obtaining a heat sensitive element by spray-coating**
Verfahren zur Herstellung eines wärmeempfindichen Elements durch Sprühbeschichtung
Procédé de fabrication d'un élément thermosensible avec revêtement par pulvérisation

(43) Date of publication of application: 21.03.2001
(73) Proprietor: AGFA-GEVAERT, 2640 Mortsel (BE)
(72) Inventor: Verschueren, Eric c/o Agfa-Gevaert, 2640 Mortsel (BE)

(56) References cited:
- EP-A- 0 818 711
- EP-A- 0 849 091
- US-A- 4 626 484
- US-A- 5 713 287

## Description

### FIELD OF THE INVENTION

The present invention relates to a method for preparing a heat sensitive element by spray-coating.

### BACKGROUND OF THE INVENTION.

Lithography is the process of printing from specially prepared surfaces, some areas of which are capable of accepting lithographic ink, whereas other areas, when moistened with water, will not accept the ink. The areas which accept ink form the printing image areas and the ink-rejecting areas form the background areas.

In the art of photolithography, a photographic material is made imagewise receptive to oily or greasy ink in the photo-exposed (negative working) or in the non-exposed areas (positive working) on a hydrophilic background.

In the production of common lithographic plates, also called surface litho plates or planographic printing plates, a support that has affinity to water or obtains such affinity by chemical treatment is coated with a thin layer of a photosensitive composition. Coatings for that purpose include light-sensitive polymer layers containing diazo compounds, dichromate-sensitized hydrophilic colloids and a large variety of synthetic photopolymers. Particularly diazo-sensitized systems are widely used.

Upon imagewise exposure of the light-sensitive layer the exposed image areas become insoluble and the unexposed areas remain soluble. The plate is then developed with a suitable liquid to remove the diazonium salt or diazo resin in the unexposed areas.

On the other hand, methods are known for making printing plates involving the use of imaging elements that are heat sensitive rather than photosensitive. A particular disadvantage of photosensitive imaging elements such as described above for making a printing plate is that they have to be shielded from the light. Furthermore they have a problem of sensitivity in view of the storage stability and they show a lower resolution. The trend towards heat sensitive printing plate precursors is clearly seen on the market.

For example, Research Disclosure no. 33303 of January 1992 discloses a heat sensitive imaging element comprising on a support a cross-linked hydrophilic layer containing thermoplastic polymer particles and an infrared absorbing pigment such as e.g. carbon black. By image-wise exposure to an infrared laser, the thermoplastic polymer particles are image-wise coagulated thereby rendering the surface of the imaging element at these areas ink acceptant without any further development. A disadvantage of this method is that the printing plate obtained is easily damaged since the non-printing areas may become ink accepting when some pressure is applied thereto. Moreover, under critical conditions, the lithographic performance of such a printing plate may be poor and accordingly such printing plate has little lithographic printing latitude.

**EP-A- 514 145** discloses a heat sensitive imaging element including a coating comprising core-shell particles having a water insoluble heat softenable core component and a shell component which is soluble or swellable in aqueous alkaline medium. Red or infrared laser light directed image-wise at said imaging element causes selected particles to coalesce, at least partially, to form an image and the non-coalesced particles are then selectively removed by means of an aqueous alkaline developer. Afterwards a baking step is performed. However the printing endurance of a so obtained printing plate is low.

**EP-A- 599 510** discloses a heat sensitive imaging element which comprises a substrate coated with (i) a layer which comprises (1) a disperse phase comprising a water-insoluble heat softenable component A and (2) a binder or continuous phase consisting of a component B which is soluble or swellable in aqueous, preferably aqueous alkaline medium, at least one of components A and B including a reactive group or precursor therefor, such that insolubilisation of the layer occurs at elevated temperature and/or on exposure to actinic radiation, and (ii) a substance capable of strongly absorbing radiation and transferring the energy thus obtained as heat to the disperse phase so that at least partial coalescence of the coating occurs. After image-wise irradiation of the imaging element and developing the image-wise irradiated plate, said plate is heated and/or subjected to actinic irradiation to effect insolubilisation. However the printing endurance of a so obtained printing plate is low.

**EP-A- 625 728** discloses an imaging element comprising a layer which is sensitive to UV- and IR-irradiation and which can be positive or negative working. This layer comprises a resole resin, a novolac resin, a latent Bronsted acid and an IR-absorbing substance. The printing results of a lithographic plate obtained by irradiating and developing said imaging element are poor.

**US-P- 5 340 699** is almost identical with **EP-A- 625 728** but discloses the method for obtaining a negative working IR-laser recording imaging element. The IR-sensitive layer comprises a resole resin,a novolac resin, a latent Bronsted acid and an IR-absorbing substance. The printing results of a lithographic plate obtained by irradiating and developing said imaging element are poor.

**US-P- 4 708 925** discloses a positive working imaging element including a photosensitive composition comprising an alkali-soluble novolac resin and an onium-salt. This composition can optionally contain an IR-sensitizer. After image-wise exposing said imaging element to UV - visible - or eventually IR-radiation followed by a development step with an aqueous alkali liquid there is obtained a positive working printing plate. The printing results of a lithographic plate obtained by irradiating and developing said imaging element are poor.

**EP-A- 800 929** discloses a heat sensitive imaging element comprising on a hydrophilic surface of a lithographic base an image forming layer comprising hydrophobic thermoplastic polymer particles dispersed in a water insoluble alkali soluble or swellable resin and a compound capable of converting light into heat, said compound being present in said image forming layer or a layer adjacent thereto, wherein said alkali swellable or soluble resin comprises phenolic hydroxy groups and/or carboxyl groups. However by exposure with short pixel times of said heat-sensitive imaging element there occurs ablation on the exposed areas resulting in an insufficient ink acceptance.

Analogous imaging elements comprising on a hydrophilic surface of a lithographic base an image forming layer comprising hydrophobic thermoplastic polymer particles dispersed in a water or alkali soluble or swellable resin and a compound capable of converting light into heat, said compound being present in said image forming layer or a layer adjacent thereto are disclosed in e.g.
**EP-A-770 494, EP-A-770 495, EP-A-770 496, EP-A-770 497,**
**EP-A-773 112, EP-A-773 113, EP-A-774 364, EP-A-800 928, EP-A-832 739, EP-A-839 648, EP-A-839 647** and **EP-A-849 091.** In most of these applications poly(meth)acrylate latices are used as thermoplastic polymer particles and no specific hydrophilic resin is mentioned In most cases carbon black or an IR-dye are mentioned as the compound capable of converting light into heat.

**US-P-5 713 287** describes a direct-to-press system using a seamless cylinder onto which a curable polymer is spray coated on the press.

In order to prepare an imaging element as described above, that is processable on the press, preferably IR-dyes should be used. Carbon black causes indeed a soiling on the press when removing the unexposed areas. On the other hand when using IR-dyes the unexposed areas are not completely dissolved when developing on the press resulting in scumming.

The appliance of the coatings which are used at the preparation of lithographic precursor plates happens mostly with coating techniques such as dipcoating, cascade coating and curtain coating. The use of spray techniques for applying lithographic layers fails usually at the attainable level of cosmetic quality of the end product. The conditions for high qualitative lithographic materials (thermal printing plates well or not processable on press) whereat high resolution, sensitivity and reproducing characteristics are required, are very high with relation with the cosmetic quality of said printing plate. This cosmetic quality can be translated as the presence of lines, the general evenness and the presence of a mottle pattern. This mottle pattern appears at the slighest presence clearly in the printing process of large screen planes.

### OBJECTS OF THE INVENTION.

It is an object of the present invention to provide the necessary parameters for obtaining a spray-coated layer with excellent cosmetic quality.

### SUMMARY OF THE INVENTION

According to the present invention there is provided a method for obtaining a high quality printing plate by spraying a spray solution on a receiving surface of grained and anodized aluminum, characterized in that the spray factor (SF) is between 48 and 70 mN/m, wherein$\text{SF = (P/d)x σ}$
SF: Spray Factor (mN/m)
P: Spray Profile (mm)
d: distance between spray head and receiving surface (mm)
σ: surface tension (mN/m).

### DETAILED DESCRIPTION OF THE INVENTION.

To define the spray profile, under well defined settings from solution and hardware , during 1 pass of the rotating drum, a line is sprayed without transverse movement of the spray head. To obtain the right spray pattern, as substrate a well swelling receiving layer, comprising gelatin, polyvinylpyrrolidone and polyethylene glycol ( Agfajet Photograde paper HP Glossy 165™, commercially available from Agfa-Gevaert) was used. This results in an immediate freezing of the spray pattern without the possibility of transverse flowing of the spray solution over the receiving surface. From this line, with the use of microdensitometry, the density profile of the line is measured. In the next step, the width at half height of this profile is divided by the total height (the maximum density) of the profile. This value is referred as profile value (P).

This profile value is determined by the air pressure of the spraying head, by the flow rate of the spraying head and by the nature of the receiving surface.

This value lies preferably between 50 and 220 mm although this value has to be considered in the context of the given equation. The surface tension of the spray solution lies preferably between 22 mN/m and 60 mN/m.

The distance between the spray head and the receiving member lies preferably between 25 and 100 mm.

The spray solution is preferably an aqueous solution, which may comprises surfactants, preferably fluorosurfactants. The viscosity of the spraying solution is preferably at least 1.5 mPa.s.

The receiving surface can be a drum with a hydrophilic surface, which can be incorporated in a printing machine.

The receiving surface can be a lithographic surface mounted on a drum.

The following spray settings results in optimum coating quality:
Drum speed: 200-240 rpm
Distance spray head: 60-100 mm
Flow rate: 6-8 ml/min
Air pressure: 5.17x10 ⁵-7.24x10 ⁵ Pa
Number of coatings : 5-7
Speed of spray head 1-2 m/min
Drying temperature: 70°C
Type spray head: air assisted SUJ1

A preferred spraying solution is a dispersion of hydrophobic thermoplastic polymer particles in a hydrophilic binder.
Said solution preferably includes thermoplastic particles of a homopolymer or a copolymer of styrene and a hydrophilic polymer containing carboxyl groups, and further a compound capable of converting light into heat.
Such solutions, suitable for spraying heat sensitive imaging elements are described with their exposure and development in **EP-A- 98 200 187.**

The receiving element is a lithographic base with a hydrophilic support, namely an anodized roughened aluminum support.

The imaging element, obtained by spraying the spray solution on the receiving element can after exposure to an IR-laser be developed by rinsing the element with an aqueous solution. Preferably the exposed imaging element is mounted directly on the press.

The following examples illustrate the present invention without limiting it thereto. All parts and percentages are by weight unless otherwise specified.

### Examples

### Preparation of spray sollution

### Spray solution A

A 2.61 wt solution in water was prepared by mixing polystyrene latex, dye I and a hydrophilic binder. After spraying and drying, the resulting layer contained 75% W/W of the polystyrene latex, 10% of the dye A and 15%W/W of Glascol E 15™. Glascol E 15 is a polyacrylic acid, commercially available at N.V. Allied Colloids Belgium.
The structure of Dye I is as follows.

### Spray solution B

To spray solution A, 5 ml of a fluorosurfactant was added.

### Spray solution C

To spray solution A, 10 ml of a fluorosurfactant was added.

### Example 1

### Preparation of the lithographic base

A 0.30 mm thick aluminum foil was degreased by immersing the foil in an aqueous solution containing 5 g/l of sodium hydroxide at 50°C and rinsed with demineralized water. The foil was then electrochemically grained using an alternating current in an aqueous solution containing 4 g/l of hydrochloric acid, 4 g/l of hydroboric acid and 5 g/l of aluminum ions at a temperature of 35°C and a current density of 1200 A/m² to form a surface topography with an average center-line roughness Ra of 0.5 mµ.

After rinsing with demineralized water the aluminum foil was then etched with an aqueous solution containing 300 g/l of sulfuric acid at 60°C for 180 seconds and rinsed with demineralized water at 25°C for 30 seconds.

The foil was subsequently subjected to anodic oxidation in an aqueous solution containing 200 g/l of sulfuric acid at a temperature of 45°C, a voltage of about 10 V and a current density of 150 A/m² for about 300 seconds to form an anodic oxidation film of 3.00 g/m² of Al₂O₃, then washed with demineralized water and posttreated with a solution containing polyvinylphosphonic acid and subsequently with a solution containing aluminum trichloride, rinsed with demineralized water at 20°C during 120 seconds and dried.

### Preparation of the heat-mode imaging element

On above mentioned lithographic base was sprayed spray solution A. Therefore, the lithographic base was mounted on a drum, rotating at a line speed of 164 m/min. The imaging element was coated by a spray nozzle moving in transverse direction at a speed of 1.5 m/min. The spray nozzle was mounted on a distance of 80 mm between nozzle and receiving substrate. The flow rate of the spray solution was set to 7 ml/min. During the spray process an air pressure of 7.58x10 ⁵ Pa was used on the spray head. The final coat weight is obtained by sequencely spraying during 6 passes of the spray head. This layer was dried on a temperature of 70°C during the spraying process and additionally during 30 s. The spray nozzle was of the type SUJ1, an air assisted spray nozzle, commercially available at Spraying Systems Belgium, Brussels

### Example 2

The same base was used as described in example 1

### Preparation of the heat-mode imaging element

The same spray solution and procedure was used as described in example 1 except following settings: the flow rate of spray solution was set to 4 ml/min and air pressure was set to 6.21x10 ⁵ Pa.

### Example 3

### The same base was used as described in example 1

### Preparation of the heat-mode imaging element

The same spray solution and procedure was used as described in example 1 except following settings:
the distance between spray nozzle and receiver was set to 60 mm and air pressure was set to 6.21x10 ⁵ Pa.

### Example 4

The same base was used as described in example 1

### Preparation of the heat-mode imaging element

The same spray solution and procedure was used as described in example 2 except following settings: the flow rate of spray solution was set to 15 ml/min.

### Example 5

### The same base was used as described in example 1

### Preparation of the heat-mode imaging element

The same spray solution and procedure was used as described in example 2 except following settings:
the flow rate of spray solution was set to 10 ml/min.

### Example 6

### The same base was used as described in example 1

### Preparation of the heat-mode imaging element

The same spray solution and procedure was used as described in example 3 except following settings:
the distance between spray nozzle and receiver was set to 45 mm.

### Example 7

### The same base was used as described in example 1

### Preparation of the heat-mode imaging element

The same spray solution and procedure was used as described in example 3 except following settings: the distance between spray nozzle and receiver was set to 35 mm.

### Example 8

### The same base was used as described in example 1

### Preparation of the heat-mode imaging element

Spray solution B was sprayed following the procedure as described in example 1 except the setting of an air pressure of 6.21x10 ⁵ Pa instead of 7.58x10 ⁵ Pa.

### Example 9

### The same base was used as described in example 1

### Preparation of the heat-mode imaging element

Spray solution B was sprayed following the procedure as described in example 8 except the setting of an air pressure of 3.45x10 ⁵ Pa instead of 6.21x10 ⁵ Pa.

### Example 10

### The same base was used as described in example 1

### Preparation of the heat-mode imaging element

Spray solution B was sprayed following the procedure as described in example 9 except the setting of an air pressure of 4.83x10 ⁵ Pa instead of 3.45x10 ⁵ Pa and a reduced distance between spray nozzle and receiver of 70 mm.

### Example 11

### The same base was used as described in example 1

### Preparation of the heat-mode imaging element

Spray solution C was sprayed following the procedure as described in example 9.

### Example 12

### The same base was used as described in example 1

### Preparation of the heat-mode imaging element

Spray solution C was sprayed following the procedure as described in example 1 with a changed air pressure setting to 4.83x10 ⁵ Pa.

### Example 13

### The same base was used as described in example 1

### Preparation of the heat-mode imaging element

Spray solution C was sprayed following the procedure as described in example 1.

### Surface tension of spray solutions

The surface tension of the spray solutions was measured by the common known Wilhelmy plate method. In this method the surface tension is calculated from the measured force to disrupt the contact between a platinum plate and the liquid surface.

| Spray Solution | Surface Tension (σ) |
|---|---|
| A | 56 mN/m |
| B | 34 mN/m |
| C | 27 mN/m |

### Calculation of Spray factor

The spray factor (SF) is calculated by dividing the profile (P) by the distance between spray head and receiver in mm (d), followed by multiplication by the surface tension (σ) of the spray solution.

| Example | P | d | P/d | σ | SF |
|---|---|---|---|---|---|
| 1 | 70 | 80 | 0.875 | 56 | 49.0 |
| 2 | 90 | 80 | 1.125 | 56 | 63.0 |
| 3 | 51 | 60 | 0.844 | 56 | 47.3 |
| 4 | 103 | 80 | 1.288 | 56 | 72.1 |
| 5 | 55 | 80 | 0.688 | 56 | 38.5 |
| 6 | 38 | 45 | 0.833 | 56 | 46.7 |
| 7 | 157 | 35 | 4.485 | 56 | 251.2 |
| 8 | 124 | 80 | 1.550 | 34 | 52.7 |
| 9 | 91 | 80 | 1.137 | 34 | 38.6 |
| 10 | 57.75 | 60 | 0.962 | 34 | 32.7 |
| 11 | 144 | 80 | 1.800 | 27 | 48.6 |
| 12 | 190 | 80 | 2.375 | 27 | 64.1 |
| 13 | 269 | 80 | 3.362 | 27 | 90.7 |

### Cosmetic quality

The plates after spraying and drying are inspected visually and given a quotation in respect to the occurence of lines, uniformity level and mottle behaviour

In this procedure, the lower the value, the better the quality. A value of 0 represents a perfect quality. On the other hand a value of 5 represents a very bad quality.

For both the occurence of lines and for uniformity, a value of 1 is still acceptable. For the mottle behaviour a value of 1 is unacceptable since this mottle is visualised in large screen planes in the printing process.

| Example | SF | Cosmetic Quality | | |
|---|---|---|---|---|
| | | Lines | Uniformity | Mottle |
| 1 | 49.0 | 1 | 0.5 | 0.5 |
| 2 | 63.0 | 0.5 | 1 | 0 |
| 3 | 47.3 | 2 | 1 | 0 |
| 4 | 72.1 | 3 | 3 | 4 |
| 5 | 38.5 | 0.5 | 0.5 | 2 |
| 6 | 46.7 | 3 | 1 | 1 |
| 7 | 251.2 | 3 | 1 | 0 |
| 8 | 52.7 | 0.5 | 0 | 0 |
| 9 | 38.6 | 1 | 1 | 1 |
| 10 | 32.7 | 2 | 1 | 1 |
| 11 | 48.6 | 0.5 | 0.5 | 0.5 |
| 12 | 64.1 | 0.5 | 0 | 0.5 |
| 13 | 90.7 | 1 | 0.5 | 1 |

## Claims

1. A method for obtaining a high quality printing plate by spraying a spray solution on a receiving surface of grained and anodized aluminum, **characterized in that** the spray factor (SF) is between 48 and 70 mN/m, wherein$\text{SF = (P/d) x σ}$
SF: Spray Factor (mN/m)
P: Spray Profile (mm)
d: distance between spray head and receiving surface (mm)
σ: surface tension (mN/m)
and wherein the spray profile is determined by dividing the width at half height of the density profile of a line obtained by spraying the spray solution during one pass of the rotating drum without transverse movement of the spray head onto a substrate which immediatly freezes the spray pattern without transverse flowing by the total height of the density profile.

2. A method according to claim 1 wherein the spray solution is an aqueous solution.

3. A method according to claim 1 or 2 wherein the spray solution comprises hydrophobic thermoplastic polymer particles and a compound capable of converting light into heat.

4. A method according to claim 3 wherein said solution comprises a hydrophilic binder.

5. A method according to any of claims 1 to 4 wherein the receiving material is a drum with a grained and anodized aluminum surface, capable of being incorporated in a printing machine.

6. A method according to any of claims 1 to 5 wherein the receiving surface is a grained and anodized aluminum surface mounted onto a drum.

7. A method according to any of claims 1 to 6 wherein the spray solution has a viscosity of at least 1.5 mPa.s.

## Patentansprüche

1. Ein Verfahren zum Erhalten einer hochqualitativen Druckplatte durch Aufspritzen einer Spritzlösung auf eine Empfangsoberfläche aus gekörntem und eloxiertem Aluminium, **dadurch gekennzeichnet, daß** der Spritzfaktor (SF) zwischen 48 und 70 Nm liegt, wobei$\text{SF = (P/d) x σ}$
SF : Spritzfaktor (mN/m)
P : Spritzprofil (mm)
d : Abstand zwischen dem Spritzkopf und der Empfangsoberfläche (mm)
σ : Oberflächenspannung (mN/m),
und **dadurch gekennzeichnet, daß** zur Bestimmung des Spritzprofils die Breite bei halber Höhe des Dichteprofils einer Linie, die durch Aufspritzen der Spritzlösung auf ein Substrat während 1 Lauf der Drehwalze ohne Quervorschub des Spritzkopfes erhalten wird, durch die Gesamthöhe des Dichteprofils geteilt wird, wobei das Substrat ein sofortiges Gefrieren des Spritzmusters ohne Gefahr von Querspreitung der Spritzlösung sichert.

2. Verfahren nach Anspruch 1, **dadurch gekennzeichnet, daß** die Spritzlösung eine wäßrige Lösung ist.

3. Verfahren nach Anspruch 1 oder 2, **dadurch gekennzeichnet, daß** die Spritzlösung hydrophobe thermoplastische Polymerteilchen und eine Verbindung, die Licht in Wärme umzuwandeln vermag, enthält.

4. Verfahren nach Anspruch 3, **dadurch gekennzeichnet, daß** die Lösung ein hydrophiles Bindemittel enthält.

5. Verfahren nach einem der Ansprüche 1 bis 4, **dadurch gekennzeichnet, daß** das Empfangsmaterial eine Trommel mit einer gekörnten und eloxierten Aluminiumoberfläche ist, die in eine Druckmaschine eingespannt werden kann.

6. Verfahren nach einem der Ansprüche 1 bis 5, **dadurch gekennzeichnet, daß** die Empfangsoberfläche eine auf eine Trommel aufgespannte gekörnte und eloxierte Aluminiumoberfläche ist.

7. Verfahren nach einem der Ansprüche 1 bis 6, **dadurch gekennzeichnet, daß** die Spritzlösung eine Viskosität von zumindest 1,5 mPa.s aufweist.

## Revendications

1. Procédé de confection pour plaque d'impression de qualité par l'étape consistant à pulvériser une solution de pulvérisation sur une surface réceptrice d'aluminium grainé et anodisé, **caractérisé en ce que** le facteur de pulvérisation (SF) est compris entre 48 et 70 mN/m, où$\text{SF = (P/d) x σ}$
SF: facteur de pulvérisation (mN/m)
P: profil de pulvérisation (mm)
d: distance entre la tête de pulvérisation et la surface réceptrice (mm)
σ: tension superficielle (mN/m)
et où le profil de pulvérisation est calculé en divisant la largeur à mi-hauteur du profil de densité d'une ligne obtenue par la pulvérisation de la solution de pulvérisation sur un substrat pendant une seule passe du tambour rotatif sans déplacement transversal de la tête de pulvérisation, ledit substrat congélant le motif de pulvérisation immédiatement sans écoulement transversal, par la hauteur totale dudit profil de densité.

2. Procédé selon la revendication 1, **caractérisé en ce que** ladite solution de pulvérisation est une solution aqueuse.

3. Procédé selon la revendication 1 ou 2, **caractérisé en ce que** ladite solution de pulvérisation comprend des particules polymères thermoplastiques hydrophobes et un composé apte à transformer de la lumière en chaleur.

4. Procédé selon la revendication 3, **caractérisé en ce que** ladite solution comprend un liant hydrophile.

5. Procédé selon l'une quelconque des revendications 1 à 4,
**caractérisé en ce que** le matériau récepteur est un tambour à surface d'aluminium grainé et anodisé, apte à être incorporé à une machine d'impression.

6. Procédé selon l'une quelconque des revendications 1 à 5, **caractérisé en ce que** ladite surface réceptrice est une surface d'aluminium grainé et anodisé accrochée sur un tambour.

7. Procédé selon l'une quelconque des revendications 1 à 6, **caractérisé en ce que** ladite solution de pulvérisation possède une viscosité d'au moins 1,5 mPa.s.
